

T. S. MAFFITT.

APPARATUS FOR TREATING IRON ORES PREPARATORY TO MAGNETIC SEPARATION.

APPLICATION FILED JULY 9, 1914.

1,295,780.

Patented Feb. 25, 1919.

2 SHEETS—SHEET 1.

Fig. I.



## *Witnesses*

J. H. Newham

E. L. Greenwald

*Inventor:*

Thomas S. Maffitt

by Foster Fauman Nathan & Co.  
**Attorneys:**

T. S. MAFFITT.

APPARATUS FOR TREATING IRON ORES PREPARATORY TO MAGNETIC SEPARATION.

APPLICATION FILED JULY 9, 1914.

1,295,780.

Patented Feb. 25, 1919.

2 SHEETS-SHEET 2.



## *Witnesses*

*R. H. Newham*

W. Greenwald.

*Inventor:*

Thomas S. Maffitt

Thomas S. Maffitt  
by Foster Freeman Watson & Co.

*Attorneys:*

# UNITED STATES PATENT OFFICE.

THOMAS S. MAFFITT, OF ST. LOUIS, MISSOURI, ASSIGNOR, BY MESNE ASSIGNMENTS, TO MISSISSIPPI VALLEY IRON COMPANY, OF WILMINGTON, DELAWARE, A CORPORATION OF DELAWARE.

## APPARATUS FOR TREATING IRON ORES PREPARATORY TO MAGNETIC SEPARATION.

1,295,780.

Specification of Letters Patent.

Patented Feb. 25, 1919.

Original application filed May 9, 1910, Serial No. 560,329. Divided and this application filed July 9, 1914. Serial No. 850,002.

*To all whom it may concern:*

Be it known that I, THOMAS S. MAFFITT, a citizen of the United States, residing at St. Louis, State of Missouri, have invented certain new and useful Improvements in Apparatus for Treating Iron Ores Preparatory to Magnetic Separation, of which the following is a specification.

It has been previously proposed to render non-magnetic iron ores magnetic by subjecting the same to a reducing agent as a hydrocarbon gas, but the treated ore has always been reduced to ordinary outside temperature before it was passed through a magnetic separator.

I have discovered that by subjecting the ore to magnetic separation while hot at a temperature considerably above normal, ores can be separated which cannot be separated at all by the process outlined above.

The process generally stated consists in rendering the ore magnetic by heat treatment and separating the ore from the gangue magnetically while in a heated state.

More specifically stated the process consists in heating the ore, subjecting the same to a reducing agent, preferably a hydrocarbon, and passing the treated ore in a heated state through a magnetic separator.

In order to describe the process and the apparatus for performing the same in detail reference is had to the accompanying drawings, in which:

Figure 1 is an elevation showing the apparatus;

Fig. 2 is a longitudinal section of the reducer; and

Figs. 3 and 4 are enlarged detail sectional views of the reducer.

The apparatus generally stated consists of a calciner A, a reducer B, and a magnetic separator C. While these separate parts of the entire apparatus may be of varied construction, an illustrative form of each will be described.

The calciner consists of a long rotary drum which is supported upon rolls 10 and is driven by means of intermeshing gears driven from a pulley 11. The drum extends into an end casing 12 provided with a charging hopper 13 and into an end casing 14 provided with a discharge chute 15. A suit-

able pipe 16 extends into the head 14 and terminates in a burner whereby heat may be supplied to the interior of the drum. The end casing 12 has connected thereto a fan 17 by means of which a current of air may be drawn through the drum so as to pass a blast of air past the burner and through the drum from one end to the other. The specific calciner has been described in the patent of Edward F. Goltra, 961,121, dated June 14, 1910.

The reducer consists of a long inclined cylinder composed of sections 20 and 21 of different diameters and supported by means of antifriction rolls 22. This drum is rotated by means of intermeshing gears driven by means of a pulley 23. The drum sections are lined with a heat resisting lining and have longitudinal ribs 24 and 25 formed thereon. The upper end of the drum extends into a stationary portion 26 which has mounted thereon a filling hopper 26<sup>a</sup> and is provided with a hinged gate or closure 27. The lower end of the drum extends into an end portion 32 which is provided with a discharge chute 28 closed by a hinged gate or closure 29.

A device 30 for feeding a suitable reducing agent to the apparatus extends longitudinally thereof and comprises an outside pipe 31 suitably supported in the end 32 and in spiders 33. A pipe 34 is located inside of the pipe 31 and is of smaller diameter so as to leave a free space between them. A third pipe 35 is located inside of the pipe 34 and is of smaller diameter so as to leave a free space between the pipes 34 and 35. In order to separate the different pipes a series of spacing blocks *a* are provided. The intermediate pipe 34 is open at its end but the outside pipe 31 is closed and the pipe 35 extends through the closed end 36 and forms a tight joint therewith. The pipe 35 is connected to a suitable reservoir containing a reducing agent as crude oil or any other hydrocarbon compound. The pipes 31 and 34 form together a water jacket for the feed pipe 35, the water being admitted at 37 and discharged through pipe 38.

The lower end 40 of the drum is not provided with a heat resisting lining but is bare, and a spray pipe 41 is arranged to direct a spray of water on the part 40 so as to cool

the same. The water spray is caught by a pan 42 arranged underneath the drum.

The magnetic separator C may be of any suitable construction. In this case it is of the Wenstrom type.

The ore is admitted to the hopper 13 and passed through the drum A and is there subjected to a heat treatment by means of the hot blast passing through the drum. The ore as it leaves the drum in a highly heated state is discharged into the hopper 26<sup>a</sup> and the drum of the reducer B. As the ore passes through the reducer drum the reducing agent, which in this case is crude oil, is admitted through the pipe 35 and as it drops on the heated ore is converted into a gas. It will be noted that the end 20 of the drum is of larger diameter than the end 21. The upper end of the cylinder is of large diameter so as to furnish a large volume for the hydrocarbon gases to act on the material. The lower end of the cylinder, or rather the lower half, is reduced in diameter so as to form a small outlet, thereby preventing entrance of air. As the ore is tumbled around in the drum all parts of the ore will be thoroughly subjected to the generated gas and will thus be rendered magnetic. As this ore reaches the lower end 40 of the drum it is cooled to some extent by the spray of water from the pipe 41. The ore in a heated state is discharged directly into the hopper 43 of the magnetic separator C and is then separated from its gangue. During the reducing operation the free access of air to the interior of the reducer apparatus must be prevented and it is for this purpose that the hinged valves or gates 27 and 29 are provided. These valves allow free admission and discharge of the ore but at the same time prevent free access of air.

The ore as it leaves the calciner will be highly heated, frequently as high as 2000° F., and the ore as discharged from the reducer will still be at a comparatively high temperature. The temperature at which the ore must be separated will vary somewhat, but I have found that for calcined brown hematite containing originally large percentages of clay gangue that the ore begins to lose its susceptibility to a magnetic field at 450° F. and below that temperature loses it very quickly, so that at ordinary temperatures it is practically non-magnetic. However if the temperature is kept above the critical point, which seems to be 450° F. for calcined brown hematite, the ore is found to be magnetic so that it can be separated by a magnetic separator without trouble.

The theory upon which the operation of this invention depends cannot be stated with definiteness. The ore as it leaves the calciner analyzes  $Fe_2O_3$ , but the ore upon leaving the reducing kiln contains a distinct amount of  $Fe_3O_4$  and  $Fe_6O_7$ . However if

the ore when it leaves the reducer is allowed to cool too much it loses its magnetism, but even after it loses its magnetism it still analyzes the same as before. This result leads to the conclusion that the change is of a physical nature rather than of a chemical nature. Furthermore, in breaking open a large lump, for instance a lump two inches in diameter, it is found that the interior as you go toward the inside is less magnetic than the outside. It is also found that the magnetism penetrates deeper into porous ore than into dense ore. This result leads to the conclusion that the action which takes place in the reducing apparatus forms what might be termed a magnetic film on the exterior of the ore sufficient to make it susceptible to a magnet while the ore is still hot. I do not however desire to be understood as advancing this theory as the only one or as being necessary, but merely one which may be advanced from the results obtained. The results show that when the iron ore is rendered magnetic by the process described and maintained above the critical temperature, which for calcined brown hematite clayey ores is 450° F., it can be efficiently separated magnetically while when the temperature drops below the critical point the ore is practically non-magnetic.

It is to be understood that the ore is cooled down in the section 40 so as to prevent injury to the magnetic separator. It seems however that the permeability increases with the temperature so that it is desirable to maintain as high a temperature as possible.

The above described apparatus may be varied to suit requirements, for instance, the rotary drum A may be replaced by another form of calcining kiln, and other types of reducers may be provided. The term "reducer" is here used to designate an apparatus for reducing the iron from a non-magnetic to a magnetic state. Generally this is accomplished by a reducing gas.

This process is especially useful and convenient when used in connection with the process described in the above mentioned patent of Edward F. Goltra. In the above application the clay iron ore is passed through the drum and heated by the hot blast, tumbled and agitated so as to shake loose the gangue from the ore, and subjected to the hot blast so as to sweep and clean the gangue from the ore.

Now it is found that in the operation of such an apparatus it will sometimes happen that the clay will be burnt to a brick, causing the formation of "clay balls." This happens when the operator is careless in applying the blast or when the drum is not long enough, or when the material is sent through the drum at too great a rate.

By passing the ore discharged from the calciner A through the reducer B the ore is

rendered magnetic and then can be easily separated from the clay balls or from the remaining clay by means of the magnetic separator.

- 5 Instead of utilizing the reducer and the magnetic separator for separating the clay balls from the ore, it is possible to perform this step of the process in other ways, for instance by means of suitable jigs. A suitable apparatus for this purpose is the well known Bradford jig. In both of the methods enumerated however, the ore is prepared in the previous step for operation in the succeeding step of the process.
- 10 15 No claim is herein made to the process described which latter forms the subject matter of a separate application, viz. Serial No. 560,329, filed May 9, 1910 of which this application is a division.
- 20 25 It is obvious that various changes may be made without departing from the spirit of this invention and it is therefore to be understood that this invention is not to be limited to the specific arrangements or construction shown and described.

Having thus described the invention what is claimed as new is:

1. In an apparatus for treating ores preparatory to magnetic separation, a drum 30 having admission and discharge openings and adapted to pass the ore therethrough, the cross section of said drum being greater at the ore admission end than at the ore discharge end, and means for maintaining an atmosphere in said drum adapted to render the ore magnetic.
2. In an apparatus for treating ores preparatory to magnetic separation, a drum comprising a section of comparatively large 40 diameter provided with an ore admission opening and a section of comparatively small diameter provided with a discharge opening, means for supporting said drum for rotation adapted to pass ore therethrough, and 45 means for maintaining an atmosphere in said drum adapted to render the ore magnetic.

3. In an apparatus for treating ores preparatory to magnetic separation, a drum having admission and discharge openings 50 and adapted to pass the ore therethrough, the cross section of said drum being greater at the admission end than at the discharge end, means for maintaining an atmosphere in said drum adapted to render the ore magnetic, and ore inlet and outlet closures for said drum adapted to seal said drum.

4. In an apparatus for treating ores preparatory to magnetic separation, a drum having admission and discharge openings 60 and adapted to pass the ore therethrough, the cross section of said drum being greater at the admission end than at the discharge end, means for maintaining an atmosphere in said drum adapted to render the ore magnetic, and means for directing a cooling spray on the discharge end of said drum.

5. In an apparatus for treating ores preparatory to magnetic separation, an inclined drum having an inlet and an outlet and 70 adapted to permit the ore to pass therethrough, means for rotating said drum, and a pipe extending along said drum and adapted to discharge a reagent on the ore to become vaporized thereby so as to create in 75 said drum an atmosphere adapted to render the ore magnetic.

6. In an apparatus for treating ores preparatory to magnetic separation, an inclined drum having an inlet and an outlet and 80 adapted to permit the ore to pass therethrough, means for rotating said drum, and a jacketed pipe extending along said drum and adapted to discharge a reagent on the ore to become vaporized thereby so as to 85 create in said drum an atmosphere adapted to render the ore magnetic.

In testimony whereof I affix my signature in presence of two witnesses.

THOMAS S. MAFFITT.

Witnesses:

EDWARD F. GOLTRA,  
J. D. DANA.